

Jan. 20, 1942.

E. W. BOEHNE

2,270,723

ARC SHIELD

Filed Aug. 1, 1940

Fig. 1.



Fig. 2.



Fig. 3.



Inventor:  
 Eugene W. Boehne,  
 by Harry C. Dunham  
 His Attorney.

## UNITED STATES PATENT OFFICE

2,270,723

ARC SHIELD - *HC + asbestos*Eugene W. Boehne, Drexel Hill, Pa., assignor to  
General Electric Company, a corporation of  
New York

Application August 1, 1940, Serial No. 349,305

9 Claims. (Cl. 200—144)

This invention relates to improved cemented asbestos arc shields or chute structures commonly used in blow out devices, such as magnetic or gas blast circuit breakers, to confine and extinguish the arc drawn between the opening electrical contacts of such devices.

One type of arc chute to which this invention particularly relates is shown and described in a copending application, Serial No. 298,946, filed October 11, 1939, in the name of Leonard J. Linde, and assigned to the same assignee as the present invention. In such a chute the arc is confined in a relatively small space, during the extinguishment thereof, and it is important that the chute be made of some heat-resistant material which will aid in the interruption of the circuit by cooling the arc to extinguishing temperatures. Such chutes or portions thereof are commonly made from various inorganic mixtures, for example, they may be made by molding a moistened mixture comprising a Portland cement binder and asbestos into the desired final shape and thereafter allowing the cement to harden in the desired form or by machining a block or board of suitable dimensions composed of such hardened cement-asbestos mixtures to the desired shape and size.

The use of cement-asbestos compositions for this purpose has a number of advantages including low material cost, ease of manufacture, and ability of the finished shields to resist sudden temperature changes. However, even after thorough drying, cement-asbestos shields or chutes have not always proven entirely satisfactory in so far as their arc interrupting ability has been concerned.

It is, therefore, an object of this invention to provide cement-asbestos chute structures of increased interrupting capacity capable of interrupting currents of higher values than previous structures of similar type.

It is a further object to provide an arc shield or chute with surfaces capable of resisting the effects of high temperature arcs and capable of imparting a greater arc-interrupting capacity to the structure.

According to the present invention the above objects and others, which will become apparent to those skilled in the art from the following description of the invention, are attained by subjecting those surfaces of the arc shields or chutes contacted by the arc during the interruption thereof to a vitrification, for example, by subjecting the surfaces to a suitable intense heating agency, such as an electric arc or a gas

flame or other means for producing at least a partial fusion of these surfaces.

For a better understanding of my invention, reference may be had to the accompanying drawing in which Fig. 1 illustrates a partial sectional view of an arc chute embodying my invention similar to the arc chute disclosed in the copending application referred to above, Fig. 2 is a cross-sectional view taken on line 2—2 of Fig. 1, and Fig. 3 is an enlarged view suitably labeled of a portion of Fig. 2 to illustrate my invention better.

In Fig. 1, I have illustrated a circuit breaker similar to that disclosed in the copending application referred to above comprising an arc chute 10 associated with which is a pair of relatively movable contacts, not shown. Relative movement between these contacts is obtained by means of an operating mechanism generally indicated at 11. The arc chute 10 comprises spaced side walls 12 composed of arc-resisting material, each side wall 12 having on the side facing the other wall a plurality of parallel fins 13 integral with the side walls, which walls 12 are suitably clamped together by means of members 14 and bolts 15 to form a chutelike structure perpendicular with the fins extending into the chute opening in staggered interleaved relation with respect to each other as best shown in Figs. 2 and 3.

One method by which the invention may be carried into effect includes subjecting the chute surfaces to the effects of a high temperature arc of brief duration in their assembled position within the breaker structure. Preferably the arc should be of greater intensity than that which the chute will ordinarily encounter in actual use. It is desirable that the duration of this treatment be rather short, preferably of the order of 8 or 10 cycles. In this respect it may be compared with the ordinary power failure arc to which such a chute may be subjected during the opening of a line breaker. However, unless such a circuit were protected by other breakers, the initial operation of the breaker before vitrification occurs would be likely to be accompanied by disastrous results by reason of its failure to protect the line adequately while vitrification still is incomplete.

Alternatively the surface conditioning of the chute may be accomplished by subjecting the surface to the heat of an arc struck between two spaced electrodes. For example, a high temperature arc playing between two electrodes spaced approximately one inch apart may be slowly

passed back and forth over the entire inner surface of the chute; that is, the active surface of the arc shields to attain the desired fusion or vitrification of a thin surface film of the shield.

A third means for carrying out this surface treatment comprises passing an oxyacetylene flame containing an excess amount of oxygen over the entire surface of the shield to obtain a partial melting or vitrification of the surface. In the practice of this method employing an ordinary oxyacetylene torch, the chute may be periodically cooled during the treatment to prevent warpage. For example, the flame treatment may be started at the center of the chute and the flame worked back and forth along the length of the chute and towards one side until one-half of the active surface of the chute has been vitrified after which the chute is cooled immediately as by immersion in water for a period of time not exceeding 15 seconds. The remaining half of the chute is then conditioned in the same manner followed by a second cooling in water.

The water treatment used in the flame conditioning process may also be found desirable in connection with the treatment of the shield or chute with an alternating current or direct current arc playing between two closely spaced electrodes. As in both of these modifications of the subject process, the heat of the arc or the flame has ample time in which to penetrate the shield structure and cause warpage of the chute, periodic cooling is desirable. This effect is not encountered when the conditioning of the chute is carried out with the first method comprising subjecting the chute to an artificial power failure since the treatment in that instance requires only a few seconds as compared with several minutes in either of the other two cases.

With each of the modifications a somewhat glassy or vitrified surface is obtained on the surfaces of the shield. The appearance of the treated surfaces varies depending upon the type of conditioning treatment used. The intense arc conditioning treatment tends to produce a rather crinkled, cracked or mottled refractory surface containing a number of rather glassy spots thereon whereas the flame conditioned surfaces have a more uniform appearance somewhat resembling ordinary glaze.

Circuit breakers containing arc shields or chutes treated in accordance with this invention have been found to have circuit-interrupting capacities up to twice those of similar breakers equipped with untreated shields or chutes. For example, a breaker, which satisfactorily cleared currents ranging from 1200 to 8700 amperes at 2300 volts when equipped with untreated chutes, was able to clear currents ranging from 10,700 to 22,000 amperes at the same voltage when equipped with treated chutes. Breakers equipped with untreated chutes which ordinarily failed at about 72,000 kva. on a 2300 volt three-phase line, have consistently cleared 120,000 kva., the capacity of the testing equipment, when equipped with flame conditioned chutes.

Cemented asbestos arc chutes that have been subjected to both the surface conditioning treatment described herein and the reducing atmosphere heat treatment described in the copending application Serial No. 349,010, filed July 31, 1940, in the name of Nicholas F. Arone and assigned to the same assignee as the present invention have been found particularly useful in circuit breaker construction. When subjecting a shield to both treatments, it has been found that

the shield may be first heated in a hydrogen atmosphere at temperatures between 350° and 600° C. for from twenty minutes to four hours and thereafter surface conditioned or conversely the shield may be first surface conditioned and thereafter heat treated in the reducing atmosphere. For practical reasons, the latter sequence has been found preferable in the manufacture of flame conditioned shields as the hydrogen heat treatment then not only serves to improve the insulation resistance of the shields in accordance with the Arone invention but also serves to dry the chutes which have been immersed in water following the flame conditioning. As the chutes which are arc conditioned in a breaker are not subjected to the heat of the arc for such a time as to permit actual penetration of the heat into the interior of the chutes, they do not require drastic cooling and may be heat treated in an atmosphere of hydrogen either before or after the arc conditioning as desired.

What I claim as new and desire to secure by Letters Patent of the United States is:

1. An arc chute comprising a molded Portland cement-asbestos base, at least a portion of the surface of said chute being coated with Portland cement-asbestos fusion products.
2. A Portland cement-asbestos arc chute having a partially vitrified surface coating covering at least that portion of the chute surface contacted by the arc during interruption thereof.
3. An arc chute comprising a mixture of Portland cement and asbestos having a refractory coating thereon consisting of the partial vitrification product of cement and asbestos.
4. A Portland cement-asbestos arc chute having a partially glazed surface, said glaze consisting of fusion products of the chute material.
5. The method of treating a Portland cement-asbestos arc chute to improve the arc interrupting properties of the chute which comprises heating at least a portion of the surface of said chute above the fusion point of the cement-asbestos mixture.
6. The method of treating a Portland cement-asbestos arc chute to improve the arc interrupting properties of the chute which comprises heating at least a portion of the surface of said chute to at least partially vitrify the same.
7. The method of treating an arc chute comprising a formed mixture of Portland cement and asbestos to improve the arc-interrupting capacity thereof, which method comprises subjecting at least a portion of the surface of said chute to a high temperature arc for a sufficient time to form a fused surface coating on the treated portions of said chute.
8. The method of treating an arc chute comprising a formed mixture of Portland cement and asbestos to improve the arc-interrupting capacity thereof, which method comprises subjecting the surface of said chute to the action of an oxyacetylene flame until at least a partial fusion of said surface takes place.
9. The process which comprises forming a thin vitrified film on the surface of a cemented asbestos insulating material by means of an oxyacetylene flame, cooling said material in water, and heat treating said material in a reducing atmosphere consisting substantially of hydrogen at a temperature between 350° and 600° C. for a period of time between twenty minutes and four hours.

EUGENE W. BOEHNE.